

## UNITED STATES PATENT OFFICE.

RUSSELL FRANKS, OF ELMHURST, NEW YORK, ASSIGNOR TO OXWELD ACETYLENE COMPANY, A CORPORATION OF WEST VIRGINIA.

## WELDING ROD.

No Drawing.

Application filed January 21, 1926. Serial No. 82,859.

It is often desirable to provide a metal article with a point, edge surface or sheath of a metal or alloy which is harder or more resistant to wear than the metal constituting the bulk of the article. It has been proposed to use welding rods and electrodes of such compositions that hard wear-resisting metal can be deposited therefrom on any suitable base by fusing the rod or the like with the blow-pipe flame or the electric arc and suitably manipulating the fused metal. The present invention is a rod or electrode of this class.

In application Ser. No. 77,575, filed by 15 Burnham E. Field and the present applicant on December 24, 1925, there are described and claimed certain new alloys suitable as material for casting wear-resisting members. The object of the present invention is to modify the compositions described in the application referred to so that the modified compositions can be made into rods or electrodes and metal deposited therefrom by fusion to give sound and homogeneous 25 deposits of metal of good wear-resisting properties.

The constituents of the alloy described in the joint application, and their preferred proportions, are as follows:

|          | Per cent.  |
|----------|------------|
| Tungsten | 1.0 to 12  |
| Chromium | 25 to 35   |
| Carbon   | 1.0 to 3.5 |
| Boron    | 0.1 to 1.0 |

30 with the remainder principally iron. I have found that good welding alloys can be made by varying the tungsten, chromium, carbon and boron through the ranges given above, it being of course understood that each of 35 these elements tends to produce brittleness if increased to the upper limit of its range, so that maximum proportions of all the elements should not be used in a single alloy. I have found, however, that in preparing 40 alloys of the above composition for welding or other like depositing operations, it is necessary to have a regulated silicon content in the alloy, whereas silicon is not an

essential constituent if the alloy is intended for casting. With a suitably adjusted silicon content the fluidity of the molten alloy is increased and the deposited metal is homogeneous and almost completely free from the blow-holes which usually occur otherwise.

50 The silicon content should have a value within the range 0.50% to 3.0%, and the best results have been obtained with silicon between 1.0% and 1.5%.

I have also found that the content of 55 manganese in the alloy and especially its proportion to the silicon are important when the alloy is to be deposited from a rod or electrode. Manganese is advantageously added to the alloy just before casting it from the original melt as it deoxidizes the metal and increases its fluidity, and I find that a small content of manganese in the alloy renders it better adapted for welding and like depositing operations. A 60 moderate excess of manganese over the amount required to deoxidize the metal is without important effect so long as the alloy is used only for casting, but when the alloy is used for welding and like depositing operations, increasing the manganese beyond certain limits has a detrimental effect. The 65 percentage of manganese should not materially exceed that of silicon. My experiments indicate that the ratio of silicon content to manganese content should be at least 70 0.9. The best results have been obtained with a silicon: manganese ratio of 1.0 and upward. Usually the quantity of manganese required to insure satisfactory casting and 75 to impart good welding qualities will prevent the ratio from exceeding 12. The introduction of a silicon content in accordance with the invention is readily accomplished, 80 a suitable commercial silicon alloy being 85 added as in many other metallurgical operations. The finished alloy is cast into rods or electrodes of any suitable form for use 90 in welding.

I claim:

95 1. A welding rod composed of alloy con-

taining tungsten 1% to 12%, chromium 25% to 35%, boron 0.10% to 1.0%, carbon 1.0% to 3.5%, silicon at least 0.50% and not over 3.0%, and manganese in sufficient quantity to deoxidize the alloy, the ratio of silicon to manganese being at least 0.9.

5. 2. A welding rod composed of alloy containing tungsten 1% to 12%, chromium 25%

to 35%, boron 0.10% to 1.0%, carbon 1.0% to 3.5%, silicon at least 1.0% and not over 10 1.5%, and manganese in sufficient quantity to deoxidize the alloy, the ratio of silicon to manganese being at least 0.9.

In testimony whereof, I affix my signature.

RUSSELL FRANKS.